

June 24, 1930.

W. H. SPIRE ET AL

**1,767,409**

## VALVE

Filed Dec. 14, 1921



FIG. I.



FIG. 2.



FIG. 3.



FIG. 4.

BY

INVENTORS:  
WILLIAM H. SPIRE  
RICHARD E. BISSELL

Amersfoort,

**ATTORNEY**

## UNITED STATES PATENT OFFICE

WILLIAM H. SPIRE AND RICHARD E. BISSELL, OF CLEVELAND, OHIO, ASSIGNEES TO  
THOMPSON PRODUCTS, INCORPORATED, OF CLEVELAND, OHIO, A CORPORATION OF  
OHIO

## VALVE

Application filed December 14, 1921. Serial No. 522,297.

This invention relates to valves, and particularly to valves used in connection with internal combustion engines.

It is the object of the invention to provide a valve which can be economically manufactured and at the same time possesses the necessary qualities of strength and resistance to the burning or oxidizing action of the heated gases with which they come into contact during use.

It is well known that cast iron possesses great durability and has excellent lasting qualities in resisting oxidation by the heated gases discharged from the cylinders in the operation of these engines. This together with the fact that cast iron can be more easily machined makes cast iron a very desirable metal for use in valve construction. Since cast iron does not possess the necessary strength for the stem of the valve, it is desirable that the stem be of steel. It is desirable that the stem be made of a non-oxidizing steel, otherwise the hot gases, often containing an excess of oxygen, escaping past the valve will oxidize the stem and soon destroy its strength. The term "non-oxidizing steel" as used herein refers, as the term is generally understood in the art, to those special steels in which a high degree of resistance to oxidation is a distinguishing characteristic. Heretofore, in attempting to integrally unite a cast iron head to a steel stem it has been found that if the stem possesses the necessary non-oxidizing qualities the strength of the stem is impaired at the joint with the head by the high heat necessary to unite the parts by fusion, and the heat treatment necessary to restore the strength of the steel stem at the joint has an injurious effect upon the cast iron head.

We have discovered that by employing a special non-oxidizing steel, the composition of which will be hereinafter specified, it is possible to integrally unite a cast iron head thereto by fusion and to restore the strength of the stem at the joint by an annealing operation which does not require a temperature high enough to injuriously affect the cast iron head.

In the annexed drawings and following description, we have set forth in detail certain means embodying our invention, the disclosed means, however, constituting but one of the various mechanical forms in which the principle of the invention may be employed.

In the annexed drawings forming a part of this specification:

Fig. 1 is a broken sectional view, showing the valve prior to the fusing together of the head and stem.

Fig. 2 is a broken sectional view, showing the valve clamped between the electrodes of a welding machine.

Fig. 3 is a broken sectional view, showing the completed valve.

Fig. 4 is a sectional view taken on the plane indicated by line IV—IV of Fig. 2.

Referring to said annexed drawings, the cast iron head 1 is drilled axially to receive the stem 2. The stem 2 has a threaded end which fits slidably in the head. To integrally unite the head and stem by fusion the head 1 is placed upon an electrode 3 formed with an opening therethrough to receive the stem and a seat 4 fitting the inner neck portion of the head. The stem is positioned with its threaded end projecting a short distance beyond the outer face of the head and with said threaded end engaging the movable electrode 5 and its opposite end engaged by a screw 6 carried by a suitably insulated stationary support 7. A suitable electric current is then passed through the electrodes and pressure is applied to the movable electrode 5. The heat due to the resistance to the passage of the current through the head and stem quickly fuses the metal and the compression on the stem upsets the threaded end of the stem within the bore of the head confining the fused metal of head and stem and causing the head and stem to be integrally united. The strength of the stem is restored by an annealing operation carried out at a comparatively low temperature and the head 1 is machined to final form as shown in Fig. 3.

A non-oxidizing steel which we have found suitable for the reason that it is capable of

being integrally united with a cast iron head and of being heat treated to restore the strength thereof without impairing said head has substantially the following composition:

|               | Per cent     |
|---------------|--------------|
| Carbon        | .50 to .60   |
| Manganese     | .30 to .50   |
| Chromium      | 7.50 to 8.50 |
| Silicon       | 1.25 to 1.75 |
| 10 Molybdenum | .60 to .90   |

The non-oxidizing property of this steel is due to its relatively high chromium content. The property which renders possible the restoration of the strength thereof by annealing at relatively low temperature is apparently due to the relatively low carbon content together with the relatively high silicon content. The best results have been obtained with steels containing these elements in percentages within the limits above specified. The small percentage of molybdenum is added to render the steel more susceptible to surface hardening treatment.

What we claim is:

1. A poppet valve for internal combustion engines consisting of a cast iron head and a stem of non-oxidizable steel and having an end portion integral with said head, the integral portion of said stem being heat-treated; the steel of such stem being of a character such as to have permitted the heat-treating at a temperature less than that which would deleteriously affect the cast iron head.

2. A poppet valve for internal combustion engines consisting of a cast iron head and a stem of non-oxidizable steel having an end portion integral with said head; the steel of said stem having a carbon content of from .5% to .6%, whereby it may be heat-treated at a temperature less than that which would deleteriously affect the cast iron head.

3. A poppet valve for internal combustion engine consisting of a cast iron head and a stem of non-oxidizable steel having an end portion integral with said head; the steel of said stem having a carbon content of from .5% to .6% and a silicon content of from 1.25% to 1.75%, whereby it may be heat-treated at a temperature less than that which would deleteriously affect the cast iron head.

Signed by us this 21st day of November, 1921.

WILLIAM H. SPIRE.  
RICHARD E. BISSELL.